# EUROPEAN PATENT SPECIFICATION

(11) **EP 0 124 026 B1**
(45) Date of publication and mention of the grant of the patent: **12.10.1988**
(21) Application number: 84104413.4
(22) Date of filing: 18.04.1984
(51) Int. Cl.: B21D 39/04, B21C 37/20

(54) **A method of forming ribs in bimetallic tubes and a ribbed tube formed by the method**
Verfahren zur Formung von Rippen an Bimetallrohren und ein nach diesem Verfahren geformtes Rippenrohr
Procédé pour former des ailettes sur des tubes bimétalliques et tube à ailettes formé selon le procédé

(30) Priority: 23.04.1983 PL 241623
(43) Date of publication of application: 07.11.1984
(73) Proprietor: Zaklady Urzadzen Chemicznych METALCHEM im. Wladyslawa Planetorza, 47-225 Kedzierzyn-Kozle (PL)
(72) Inventor: Przybyla, Janusz, PL-42-520 Zabkowice Bedzinskie (PL); Gozdziewicz, Zygmunt, PL-47-220 Kedzierzyn-Kozle (PL); Szal, Andrzej, PL-47-220 Kedzierzyn-Kozle (PL); Zub, Ryszard, PL-47-220 Kedzierzyn-Kozle (PL); Maczynski, Andrzej, PL-44-100 Gliwice (PL)
(74) Representative: Füchsle, Klaus, Dipl.-Ing.

(56) References cited:
- EP-A- 0 123 923
- DE-A- 1 452 518
- DE-B- 1 295 333
- FR-A- 932 059

## Description

This invention relates to a method of forming ribs in bimetallic tubes, in which the rib is pressed from the outer tube into which compressive prestress is previously introduced.

It is known that ribs may be formed in tubes by the action of rotary tools comprising profiled rollers. From EP-A-123923, which is cited under Art 54(3) and is not relevant to the question of inventive step, a method of pressing ribs on tubes is known, in which before placing the tube in the zone of the action of the rollers initial compressive stress is introduced into the tube. In this way relief is achieved during the operation of the tool from axial loads bending out the roll-formed disks practically from the first stage of the working contact of the tool with the tube. For the purpose of inducing compressive stresses in the tube in EP-A-123923 a screw-clamp is provided.

In the case of pressing ribs in bimetallic tubes such a solution is practically useless because it is difficult to meet the requirement of accurately setting both tubes in relation to each other with simultaneous application of a compressive force on the external tube.

From DE-A-1452518 the features of the precharacterising part of claim 1 are known.

According to the invention there is provided a method of drawing ribs on bimetallic tubes, based on the insertion of the internal tube in the external one, and drawing the ribs on the external tube by the action of disk rotary tools, is characterized in that before inserting the internal tube (1) in the external tube (2), the roughness of the external surface of the internal tube (1) is increased at two segments (P), each of a length from 0,8 to 3 d, where d denotes the external diameter of the internal tube (1), the said segments (P) being distant from each other by the value L * (1,6-6) d, where L denotes the length of the external tube (2), the internal tube (1) is placed in the external tube (2), so that the ends of the external tube (2) are in line with the outer ends of the said segments (P) of the internal tube (1) of increased roughness and next, the ends of the external tube (2) are clamped on the internal tube (1) along the length of from 0,5 to 1,5 of the length of increased roughness of the internal tube (1) at least one end of the external tube is deformed creating a simultaneous axial displacement of a part of deformed external tube (2) in the direction of the center (A) of the tube, said axial displacement being sufficiently large to cause the introduction of compressive stresses in the material of the external tube (2).

It is preferable to form at least one end of the external tube in a conical shape during clamping.

The method according to the invention enables durable connection of the external tube with the internal tube in an accurately established position of the ends of the tubes with introduction to the external tube of the necessary compressive stresses. An advantage of the method is also that merged tubes do not displace in relation to each other during rolling, and the use of instruments for the maintenance of initial stresses in the tube is eliminated to reduce labour costs of operations in the production of ribbed bimetallic tubes. Moreover, production of ribbed bimetallic tubes by this method enables considerable material savings to be achieved in relation to so-called free rolling.

The subject of the invention will be now explained in more detail with reference to the single Figure of the drawing illustrating a merged bimetallic tube with introduced initial compressive stress, prepared for forming ribs.

A bimetallic tube consists of an internal tube 1 and an external tube 2. At distances from the ends of the internal tube 1 determined by design considerations are provided segments 3 and 4 of increased roughness of the surface of the tube. The increase of roughness can be effected, for example, by knurling, grooving or thread-cutting. The length P of the segment of increased roughness is from 0.8 to 3 of the magnitude of the diameter d of the internal tube. At least one of the deformed ends of the external tube 2 is deformed so that a part of the deformed end of the tube is displaced in the axial direction, towards the centre A of the external tube 2. The quantity of the axially displaced material of the external tube 2 corresponds to the quantity of the deformation induced by introducing compressive stresses necessary for drawing the ribs.

## Claims

1. A method of drawing ribs on bimetallic tubes, based on the insertion of the internal tube in the external one, and drawing the ribs on the external tube by the action of disk rotary tools, is characterized in that before inserting the internal tube (1) in the external tube (2), the roughness of the external surface of the internal tube (1) is increased at two segments (P), each of a length from 0,8 to 3 d, where d denotes the external diameter of the internal tube (1), the said segments (P) being distant from each other by the value L * (1,6-6)d, where L denotes the length of the external tube (2), the internal tube (1) is placed in the external tube (2), so that the ends of the external tube (2) are in line with the outer ends of the said segments (P) of the internal tube (1) of increased roughness and next, the ends of the external tube (2) are clamped on the internal tube (1) along the length of from 0,5 to 1,5 ofthe length of increased roughness of the internal tube (1) at least one end of the external tube is deformed creating a simultaneous axial displacement of a part of deformed external tube (2) in the direction of the center (A) of the tube, said axial displacement being sufficiently large to cause the introduction of compressive stresses in the material of the external tube (2).

2. A method according to claim 1, characterized in that at least one end of the external tube (2) is conically formed during clamping on the internal tube (1).

## Patentansprüche

1. Verfahren zum Ziehen von Rippen auf Bimetall-Rohren, auf der Basis des Einsatzes eines Innenrohres in ein Außenrohr und Ziehen der Rippen auf dem Außenrohr durch die Wirkung von schiebenförmigen Drehwerkzeugen, dadurch gekennzeichnet, daß vor dem Einsetzen des Innenrohres (1) in das Außenrohr (2) die Rauhigkeit der äußeren Oberfläche des Innenrohres (1) in zwei Segmenten (P) erhöht wird, wobei jedes Segment eine Länge von 0,8 bis 3 d hat und d den Außendurchmesser des Innenrohres (1) bezeichnet, daß sie Segmente (P) durch einen Wert L-(1,6-6)d voneinander beabstandet sind, wobei L die Länge des Außenrohres (2) bezeichnet, daß das Innenrohr (1) so im Außenrohr (2) angeordnet ist, daß die Enden des Außenrohres (2) mit den äußeren Enden der Segmente (P) des Innenrohres (1) höherer Rauhigkeit fluchten, daß dann die Enden des Außenrohres (2) auf das Innenrohr (1) über eine Länge von 0,5 bis 1,5 der Länge erhöhter Rauhigkeit des Innenrohres (1) geklemmt werden, daß zumindest ein Ende des Außenrohres zum Erzeugen einer gleichzeitigen Axialverschiebung eines Teils des deformierten Außenrohres (2) in Richtung der Mitte (A) des Rohres deformiert wird, und daß die Axialverschiebung ausreichend groß ist, um das Einführen von Kompressionskräften im Material des Außenrohres (2) zu verursachen.

2. Verfahren nach Anspruch 1, dadurch gekennzeichnet, daß zumindest ein Ende des Außenrohres (2) während des Klemmens auf das Innenrohr (1) konisch geformt wird.

## Revendications

1. Procédé pour étirer des ailettes sur des tubes bimétalliques, reposant sur l'insertion du tube intérieur dans le tube extérieur par l'action d'outils rotatifs à disque, caractérisé en ce qu'avant d'insérer le tube intérieur (1) dans le tube extérieur (2), la rugosité de la surface extérieure du tube intérieur (1) est augmentée au niveau des deux segments (P), chaque segment ayant une longueur de 0,8 à 3 d, ou d désigne de diamètre extérieur du tube intérieur (1), les segments (P) étant distants l'un de l'autre d'une valeur de L-(1,6-6)d où L désigne la longueur du tube extérieur (2), le tube intérieur (1) est placé dans le tube extérieur (2), de sorte que les extrémités du tube extérieur (2) sont alignées sur les extrémités extérieures des segments (P) du tube intérieur (1) de rugosité accrue, et ensuite, les extrémités du tube extérieur (2) sont bridées sur le tube intérieur (1) sur la longueur de 0,5 à 1,5 de la longueur de rugosité accrue du tube intérieur (1), au moins une extrémité du tube extérieur est déformée créant un déplacement axial simultané d'une partie du tube extérieur déformé (2) dans la direction du centre (A) du tube, ce déplacement axial étant suffisamment grand pour permettre l'introduction de contraintes de compression dans le matériau du tube extérieur (2).

2. Procédé selon la revendication 1, caractérisé en ce qu'au moins une extrémité du tube extérieur (2) est formée en cône pendant le bridage sur le tube intérieur (1).
